# EUROPEAN PATENT SPECIFICATION

(11) **EP 2 835 438 B1**
(45) Date of publication and mention of the grant of the patent: **26.06.2019**
(21) Application number: 13773084.2
(22) Date of filing: 03.04.2013
(51) Int. Cl.: C21D 8/02, C21D 9/46, C22C 38/00, C22C 38/02, C22C 38/04, C22C 38/06, C25D 5/48, C25D 7/06, B22D 11/00

(54) **HIGH-STRENGTH, HIGHLY WORKABLE STEEL SHEET, AND METHOD FOR MANUFACTURING SAME**
HOCHFESTES, LEICHT ZU VERARBEITENDES STAHLBLECH UND HERSTELLUNGSVERFAHREN DAFÜR
TÔLE D'ACIER FACILEMENT FAÇONNABLE, DE RÉSISTANCE ÉLEVÉE, ET SON PROCÉDÉ DE FABRICATION

(30) Priority: 06.04.2012 JP 2012087940
(43) Date of publication of application: 11.02.2015
(73) Proprietor: JFE Steel Corporation, Tokyo, 100-0011 (JP)
(72) Inventor: TANAKA, Takumi, Tokyo 100-0011 (JP); KOJIMA, Katsumi, Tokyo 100-0011 (JP); TOBIYAMA, Yoichi, Tokyo 100-0011 (JP)
(74) Representative: Hoffmann Eitle
(86) International application number: PCT/JP2013/060175
(87) International publication number: WO 2013/151085

(56) References cited:
- EP-A1- 1 191 114
- WO-A1-2008/018531
- WO-A1-2009/123356
- JP-A- H0 533 188
- JP-A- 2001 049 383
- JP-A- 2002 146 478
- JP-A- 2002 206 138
- JP-A- 2004 218 061
- US-A1- 2003 015 263
- US-A1- 2006 228 524
- US-A1- 2011 076 177

## Description

### Field

The present invention relates to a high strength and high formability steel sheet suitable for application to a steel sheet for easy open ends of cans, and a manufacturing method thereof.

### Background

Among steel sheets used for beverage cans or food cans, a steel sheet referred to as a double reduced (DR) material may be used for lids, bottoms, bodies of three-pieced cans, drawn cans, or the like. With the DR material manufactured by a DR method of performing cold rolling again after annealing, a sheet thickness can be made thin more easily than with a single reduced (SR) material manufactured only by temper rolling after annealing at a small reduction ratio. Thus, it is possible, using the DR material, to reduce costs for manufacturing cans. In the DR method, the cold rolling performed again after annealing causes work hardening, and thus although a thin and hard steel sheet can be manufactured, its formability is less than the SR material.

As lids of beverage cans and food cans, easy open ends (EOEs) that can be opened easily are widely used. In manufacturing an EOE, it is necessary to form, by bulging, a rivet for attaching a tab with which a finger is engaged. Steel sheets as materials for manufacturing cans are required to have strengths according to sheet thicknesses, and as for the DR material, a tensile strength of not lower than about 520 MPa is necessary to ensure an economic effect due to thinning thereof. It is difficult to ensure for conventional DR materials both of formability and strength as mentioned above and thus the SR material has been used for EOEs. However, demands for applying the DR material to EOEs also are currently increasing in terms of cost reduction.

Due to such background, Patent Literature 1 discloses a steel sheet for easy open cans lids excellent in rivet formability, characterized in that its carbon content is not greater than 0.02% and its boron content is in a range of 0.010 to 0.020%, and a manufacturing method thereof, characterized in that second cold rolling is performed with a rolling reduction ratio of not greater than 30%. Moreover, Patent Literature 2 discloses a DR material characterized in that its average Lankford value after an aging treatment is not greater than 1.0, and describes that the DR material is excellent in EOE rivet formability. Patent Literature 3 discloses a high-strength steel plate for a can that has a yield stress of 500 MPa or above after coating and baking, and a method for manufacturing the same. The high-strength steel plate for a can include, by mass: over 0.02% to 0.10% carbon; 0.10% silicon or below; 1.5% manganese or below; 0.20% phosphorus or below; 0.20% sulfur or below; 0.10% aluminum or below; 0.0120% to 0.0250% nitrogen, said nitrogen including 0.0100% or more of dissolved nitrogen; with the remainder comprising iron and unavoidable impurities. A certain level or more of an absolute quantity of the dissolved nitrogen is secured, and a high-strength material can be secured by hardening through quenching aging or strain aging during the printing process, film laminating process, or drying and baking process, or the like, that is performed before the can is manufactured. When manufacturing the high-strength steel plate, the slab extraction temperature is set at 1200°C or above, hot rolling is performed at a finishing rolling temperature of (Ar3 transformation point temperature-30) °C or above, and the steel plate is coiled up at 650°C or below. The present invention differs from the teaching of Patent Literature 3 at least insofar as the thickness of the resin film layer according to the present invention is not directly and unambiguously disclosed in Patent Literature 3.

### Citation List

### Patent Literature

Patent Literature 1: Japanese Patent No. 3740779
Patent Literature 2: WO 2008/018531
Patent Literature 3: WO 2009/123356

### Summary

### Technical Problem

However, the conventional techniques described above have problems. As a diameter of a can lid to be applied becomes greater, a greater strength is required for a steel sheet, but since the steel sheet described in Patent Literature 1 has the small carbon content, the nitrogen content needs to be large to obtain a large strength. However, because the steel sheet contains at least a certain amount of boron, when the nitrogen content is large, its ductility at a high temperature becomes small and a slab crack is caused upon continuous casting. Therefore, the steel sheet described in Patent Literature 1 cannot be applied to an EOE having a large diameter.

The steel sheet described in Patent Literature 2 achieves the good rivet formability by reducing the average Lankford value. However, this method exerts its effects only when a rivet is formed by column-like bulging, and when a rivet is formed by sphere-like bulging, the rivet formability becomes insufficient. Therefore, provision of a high strength and high formability steel sheet having a tensile strength of not lower than 520 MPa and an Erichsen value of not less than 5.0 mm has been desired.

The present invention has been made in view of the above problems, and its object is to provide a high strength and high formability steel sheet having a tensile strength of not lower than 520 MPa and an Erichsen value of not less than 5.0 mm and a manufacturing method thereof, as specified in the appended claims.

### Solution to Problem

As a result of diligently performing intensive studies, the inventors of the present invention have found that it is effective, for achieving both formability and strength of a steel sheet, to ensure strength by increasing a nitrogen content while preventing deterioration of formability by restricting a carbon content to an appropriate range, and to restrict a second cold rolling reduction ratio after annealing to an appropriate range. Moreover, the inventors of the present invention have found that it is necessary to restrict also a coiling temperature to an appropriate range because, when the coiling temperature after hot rolling is high, precipitated cementite becomes coarse and local elongation deteriorates. Furthermore, the inventors of the present invention have found that rivet formability by bulging is remarkably improved by providing a resin film layer having an appropriate thickness on a side to be an inner surface of a can.

A high strength and high formability steel sheet for easy open ends of cans according to the present invention has a tensile strength in a rolling direction of not less than 520 MPa, and an Erichsen value of not less than 5.0 mm, and is obtainable by forming a slab by continuously casting a steel including, in mass%: greater than 0.020% and less than 0.040% of C; not less than 0.003% and not greater than 0.100% of Si; not less than 0.10% and not greater than 0.60% of Mn; not less than 0.001% and not greater than 0.100% of P; not less than 0.001% and not greater than 0.020% of S; not less than 0.005% and not greater than 0.100% of Al; greater than 0.0130% and not greater than 0.0170% of N; and a remainder being Fe and inevitable impurities,
performing hot rolling at a slab reheating temperature of not lower than 1150°C;
coiling at a temperature of not higher than 600°C; thereafter performing first cold rolling;
thereafter performing continuous annealing at a soaking temperature of 600 to 700°C for a soaking period of 10 to 50 seconds; and
thereafter performing second cold rolling at a reduction ratio of 8.0 to 15.0%,
the high strength and high formability steel sheet being characterized by comprising a resin film layer with a thickness of 5 to 100 µm at least on a side to be an inner surface of a can.

A thickness of the resin film layer is in a range of 5 to 100 µm.

A method of manufacturing a high strength and high formability steel sheet for easy open ends of cans according to the present invention includes: forming a slab by continuously casting a steel including, in mass%: greater than 0.020% and less than 0.040% of C; not less than 0.003% and not greater than 0.100% of Si; not less than 0.10% and not greater than 0.60% of Mn; not less than 0.001% and not greater than 0.100% of P; not less than 0.001% and not greater than 0.020% of S; not less than 0.005% and not greater than 0.100% of Al; greater than 0.0130% and not greater than 0.0170% of N; and a remainder being Fe and inevitable impurities; performing hot rolling at a slab reheating temperature of not lower than 1150°C; coiling at a temperature of not higher than 600°C; thereafter performing first cold rolling; thereafter performing continuous annealing at a soaking temperature of 600 to 700°C for a soaking period of 10 to 50 seconds; thereafter performing second cold rolling at a reduction ratio of 8.0 to 15.0%; attaching a resin film at least on a side to be an inner surface of a can after forming a surface treatment film by an electrolytic process; and manufacturing a steel sheet having a tensile strength in a rolling direction of not less than 520 MPa and an Erichsen value of not less than 5.0 mm.

### Advantageous Effects of Invention

According to the high strength and high formability steel sheet for easy open ends of cans and the manufacturing method thereof of the present invention, it is possible to obtain a high strength and high formability steel sheet having a tensile strength of not lower than 520 MPa and an Erichsen value of not less than 5.0 mm. Further, as a result, it is possible to manufacture a lid with a DR material having a small thickness, without cracking upon EOE rivet formation, and thus to achieve thinning of a steel sheet for EOEs to a great extent.

### Description of Embodiments

In the following, the present invention is described in detail.

The high strength and high formability steel sheet of the present invention is a steel sheet for easy open ends of cans having tensile strength of not lower than 520 MPa and an Erichsen value of not less than 5.0 mm.
Such a steel sheet can be manufactured with steel having carbon content of less than 0.040%, by setting a coiling temperature after hot rolling and a second cold rolling reduction ratio to appropriate conditions, and attaching a resin film on a side to become an inner surface of a can, as specified by the appended claims. In the following, the component composition of the high strength and high formability steel sheet of the present invention is described.

Component Composition of High Strength and High Formability Steel Sheet

### (1) C: Greater than 0.020% and less than 0.040%

The high strength and high formability steel sheet of the present invention exerts high formability by suppressing carbon (C) content to small. When the C content is not less than 0.040%, a steel sheet becomes excessively hard, thus making it impossible to manufacture a thin steel sheet by second cold rolling while ensuring formability. Thus, the upper limit of C content is set to be less than 0.040%. However, when the C content is not greater than 0.020%, the tensile strength of 520 MPa that is required to obtain significant economic effects resulted by thinning of a steel sheet cannot be obtained. Thus, the lower limit of C content is set to exceed more than 0.020%.

### (2) Si: Not less than 0.003% and not greater than 0.100%

When the silicon (Si) content exceeds 0.100%, there occur problems of deterioration of surface treatability, deterioration of corrosion resistance, etc. Thus, the upper limit of Si content is 0.100%. When Si content is set to be less than 0.003%, refining cost is excessively high. Therefore, the lower limit of Si content is set to be 0.003%. The preferable Si content is in a range of not less than 0.003% and not greater than 0.035%.

### (3) Mn: Not less than 0.10% and not greater than 0.60%

Manganese (Mn) has functions of preventing red shortness during hot rolling due to sulfur (S) and of refining crystal grains, and is an element necessary for ensuring the desirable quality of a material. The addition of at least 0.10% or more of Mn is required in order to exert such effects. However, when an excessive amount of Mn is added, the corrosion resistance deteriorates and a steel sheet becomes excessively hard. The upper limit of Mn amount is therefore set to be 0.60%. The preferable Mn content is in a range of not less than 0.19% and not greater than 0.60%.

### (4) P: Not less than 0.001% and not greater than 0.100%

Phosphorus (P) is a harmful element that hardens steel, and deteriorates formability, and in addition, deteriorates also corrosion resistance. Thus, the upper limit of P content is set to be 0.100%. However, when the P content is set to be less than 0.001%, the cost for dephosphorization becomes excessively high. The lower limit of P content is therefore set to be 0.001%. The preferable P content is in a range of not less than 0.001% and not greater than 0.015%.

### (5) S: Not less than 0.001% and not greater than 0.020%

S exists as inclusions in steel, and is a harmful element causing deterioration of formability and deterioration of corrosion resistance. The upper limit of S content is therefore set to be 0.020%. When the S content is set to be less than 0.001%, the cost for desulfurization becomes excessively high. The lower limit of S content is therefore set to be 0.001%. The preferable P content is in a range of not less than 0.007% and not greater than 0.014%.

### (6) Al: Not less than 0.005% and not greater than 0.100%

Aluminum (Al) is an element necessary as deoxidizer in a steelmaking process. When the Al content is small, deoxidation is insufficient, and inclusions increase, thus deteriorating formability. When the Al content is not less than 0.005%, it can be considered that deoxidation is performed sufficiently. However, when the Al content exceeds 0.100%, the frequency of occurrence of surface defects due to alumina clusters, etc. is increased. The Al content is therefore set to be not less than 0.005% and not greater than 0.100%.

### (7) N: Greater than 0.0130% and not greater than 0.0170%

In the high strength and high formability steel sheet of the present invention, nitrogen (N) content is increased, instead of reducing C content, to ensure strength. The strengthening using N has small effects on bulging formability, and thus it is possible to strengthen a steel sheet without deteriorating an Erichsen value. When N content is not greater than 0.0130%, the strength necessary for a can lid cannot be obtained. However, when a large amount of N is added, the hot ductility deteriorates, thus causing a slab crack in continuous casting. The upper limit of N content is therefore set to be 0.0170%.

### (8) Other components

The balance other than the components described above is iron (Fe) and inevitable impurities, and may include component elements normally contained in a known steel sheet for welded cans. For example, the component elements such as chromium (Cr): not greater than 0.10%, copper (Cu): not greater than 0.20%, nickel (Ni): not greater than 0.15%, molybdenum (Mo): not greater than 0.05%, titanium (Ti): not greater than 0.3%, niobium (Nb): not greater than 0.3%, zirconium (Zr): not greater than 0.3%, vanadium (V): not greater than 0.3%, calcium (Ca): not greater than 0.01%, may be contained depending on a purpose.

### Characteristics of High Strength and High Formability Steel Sheet

Next, the mechanical characteristics of the high strength and high formability steel sheet of the present invention are described.

The tensile strength of the high strength and high formability steel sheet of the present invention is set to be not lower than 520 MPa. When the tensile strength is lower than 520 MPa, a steel sheet cannot be made thin enough to obtain significant economic effects, in order to ensure the strength of the steel sheet as a material for manufacturing lids. The tensile strength is therefore set to be not lower than 520 MPa. The above tensile strength can be measured by Metallic materials-Tensile testing defined in the document "JIS Z 2241".

The Erichsen value of the high strength and high formability steel sheet of the present invention is set to be not less than 5.0 mm. When the Erichsen value is smaller than 5.0 mm, a crack occurs in rivet formation. The Erichsen value is therefore set to be not less than 5.0 mm. The Erichsen value can be measured by Method of Erichsen cupping test defined in the document "JIS Z 2247". In the rivet formation, the processing form applied on a steel sheet is bulging, which can be regarded as tensile deformation toward all directions parallel to a sheet surface. The evaluation of deformability of a steel sheet by such processing requires a test by similar bulging, and the deformability cannot be evaluated with a total elongation value or a Lankford value by the simple uniaxial tensile testing.

### Surface Coating of High Strength and High Formability Steel Sheet

Next, the surface coating of the high strength and high formability steel sheet of the present invention is described.

The rivet formation is performed by bulging, and processing for bulging toward the outer side of a can is performed. In the processing, therefore, a steel sheet is deformed by a tool contacting with the inner side surface of the can. The lubricating ability between a tool and a steel sheet is improved by contacting them with a resin film interposed therebetween. Thus, the uniformity of bulging is improved, suppressing the occurrence of a crack effectively. It is more preferable that a surface of a steel sheet be coated with a resin film in addition to interposing a resin film between a tool and a steel sheet, because those contribute to corrosion resistance.

A resin film is not particularly limited, and various thermoplastic resins and thermosetting resins can be used. For example, there may be used an olefin resin film such as of polyethylene, polypropylene, ethylenepropylene copolymer, ethylene-vinyl acetate copolymer, ethylene-acrylic ester copolymer, and ionomer, or a polyester film such as of polybutylene terephthalate, or a thermoplastic resin film including a polyamide film such as of nylon 6, nylon 6-6, nylon 11, and nylon 12, a polyvinylchloride film, and a polyvinylidene chloride film without stretching them or by stretching them biaxially.

When an adhesive is used to attach a resin film on a steel sheet, an urethane adhesive, an epoxy adhesive, an acid-modified olefin resin adhesive, a copolyamide adhesive, a copolyester adhesive (thickness: 0.1 to 5.0 µm), etc. are used preferably. Moreover, thermosetting coating is applied on the steel sheet side or the resin film side with a thickness in a range of 0.05 to 2.0 µm, and this may be regarded as an adhesive. Moreover, thermoplastic or thermosetting coating including modified epoxy coating such as of phenol epoxy and amino-epoxy, vinyl chloride-vinyl acetate copolymer, vinyl chloride acetate saponified copolymer, vinyl chloride-vinyl acetate-maleic anhydride copolymer, epoxy modified-, epoxy amino modified-, epoxy phenol modified-vinyl coating or modified vinyl coating, acryl coating, and a synthetic rubber coating such as of styrene-butadiene copolymer may be used individually or in combination of two or more thereof.

The thickness of a resin film is set to be in a range of 5 to 100 µm. When the thickness of a resin film is smaller than 5 µm, the resin film is fractured in bulging, and it is more possible that the effects are not exerted sufficiently. When the thickness of a resin film exceeds 100 µm, the effect of increasing a deformation amount of a steel sheet becomes greater, and a crack of the steel sheet will occur more easily.

### Manufacturing Method of High Strength and High Formability Steel Sheet

Next, the manufacturing method of the high strength and high formability steel sheet of the present invention is described.

The high strength and high formability steel sheet of the present invention is manufactured, with use of a steel slab having the above composition manufactured by continuous casting, by performing hot rolling at a slab reheating temperature of not lower than 1150°C, coiling it at a temperature of not higher than 600°C, performing first cold rolling, performing continuous annealing at a soaking temperature of 600 to 700°C for a soaking period of 10 to 50 seconds, performing second cold rolling with a reduction ratio of 8.0 to 15.0%, forming a surface treatment film by an electrolytic process, and then attaching a resin film at least on a side to become an inner surface of a can.

It is normally difficult, with only one-time cold rolling, to make a sheet thin enough to obtain significant economic effects. That is, in order to obtain a thin sheet with one-time cold rolling, the load on a mill becomes too high, and it is impossible to achieve it depending on a plant capacity. For example, when a final sheet thickness is made 0.15 mm, the first cold reduction ratio of as much as 92.5% is required if a sheet thickness after hot rolling is 2.0 mm. It can be also considered that a sheet is rolled to be thinner than usual at the step of hot rolling to reduce a sheet thickness after cold rolling. However, when the reduction ratio in hot rolling is increased, the reduction of a temperature of a steel sheet during rolling becomes great, and a given finish rolling temperature cannot be obtained. Moreover, when continuous annealing is performed, the possibility of the occurrence of troubles such as fracture or deformation of a steel sheet during annealing becomes higher if a sheet thickness before annealing is set to be small. For these reasons, it is preferable in the present invention that the cold rolling for the second time (second cold rolling) be performed after annealing to obtain an ultrathin steel sheet.

When a coiling temperature after hot rolling exceeds 600°C, a pearlite structure to be formed becomes coarse, which is a starting point of brittle fracture and thus reduces local elongation, making it difficult to obtain an Erichsen value of not less than 5.0 mm. The coiling temperature after hot rolling is therefore preferably not higher than 600°C, and is more preferably in a range of 550 to 600°C.

When the soaking temperature of continuous annealing is lower than 600°C or the soaking period thereof is shorter than 10 seconds, recrystallization is insufficient, thus making it difficult to obtain an Erichsen value of not less than 5.0 mm. However, when the soaking temperature exceeds 700°C or the soaking period exceeds 50 seconds, the grain growth through recrystallization becomes excessive, thus making it difficult to obtain the tensile strength of 520 MPa. The continuous annealing is therefore performed under conditions of a soaking temperature of 600 to 700°C and a soaking period of 10 to 50 seconds.

When the second cold rolling reduction ratio exceeds 15.0%, work hardening by the second cold rolling becomes excessive, thus making it difficult to obtain an Erichsen value of not less than 5.0 mm. The second cold rolling reduction ratio is therefore not greater than 15.0%. However, when the second cold rolling reduction ratio is less than 8.0%, it is difficult to obtain strength necessary for a can lid. Thus, the lower limit of the second cold rolling reduction ratio is 8.0%.

After the second cold rolling, a surface treatment film is formed by an electrolytic process. As a film, a Sn electroplating film, an electrolytic Cr acid treatment film, or the like, which is widely used for a can lid as a tin plate or tin-free steel, can be applied. The adherence between a resin film and a steel sheet can be improved by providing such a film.

After the surface treatment film is formed, a resin film is attached at least on a side to become an inner surface of a can. The attachment method can be a method of heating a steel sheet and heat-sealing a resin film, or a method of attaching it using an adhesive.

### Examples

A steel slab was obtained by melting steel having the component compositions illustrated in Table 1 and the balance including Fe and inevitable impurities in an actual converter and subjecting it to continuous casting. The obtained steel slab was heated again, and subjected to hot rolling under the conditions illustrated in Table 2. A finish rolling temperature of hot rolling was set to be 880°C, and pickling was performed after the rolling. Next, after first cold rolling was performed with a reduction ratio of 90%, continuous annealing and second cold rolling were performed under the conditions illustrated in Table 2. The electrolytic Cr acid treatment was continuously performed on the both surfaces of the steel sheet obtained in the above manner, whereby tin-free steel having a Cr coating build-up per side of 100 mg/m² was obtained. Then, an isophthalic acid copolymerized polyethylene terephthalate film having a copolymerization ratio of 12 mol% was laminated on the both surfaces, and thus a resin coated steel sheet was obtained. The laminating was performed in such a manner that a steel sheet heated to 245°C and a film were nipped by a pair of rubber covered rolls so that the film was fused to the metallic sheet, and the laminate was cooled with water within one second after it passed the rubber covered rolls. Here, a feed rate of the steel sheet was 40 m/min, and the nip length of the rubber covered rolls was 17 mm. The nip length is a length in a feed direction of a part where the rubber covered rolls and the steel sheet are in contact. The thickness of film layers was listed in Table 1.

**Table 1**

| No. | Component composition (mass%) | | | | | | | Thickness of resin layer (µm) |
|---|---|---|---|---|---|---|---|---|
| | C | Si | Mn | P | S | Al | N | |
| 1 | 0.031 | 0.011 | 0.29 | 0.009 | 0.010 | 0.039 | 0.0153 | 18 |
| 2 | 0.021 | 0.010 | 0.23 | 0.010 | 0.012 | 0.018 | 0.0161 | 24 |
| 3 | 0.039 | 0.012 | 0.25 | 0.009 | 0.010 | 0.025 | 0.0140 | 15 |
| 4 | 0.026 | 0.008 | 0.28 | 0.012 | 0.008 | 0.042 | 0.0170 | 5 |
| 5 | 0.035 | 0.009 | 0.30 | 0.013 | 0.011 | 0.048 | 0.0131 | 51 |
| 6 | 0.029 | 0.010 | 0.19 | 0.010 | 0.012 | 0.041 | 0.0148 | 100 |
| 7 | 0.020 | 0.011 | 0.26 | 0.011 | 0.009 | 0.040 | 0.0152 | 30 |
| 8 | 0.040 | 0.013 | 0.25 | 0.010 | 0.010 | 0.051 | 0.0160 | 29 |
| 9 | 0.032 | 0.012 | 0.27 | 0.009 | 0.011 | 0.044 | 0.0130 | 19 |
| 10 | 0.028 | 0.010 | 0.22 | 0.012 | 0.010 | 0.038 | 0.0175 | - |
| 11 | 0.035 | 0.014 | 0.27 | 0.010 | 0.009 | 0.033 | 0.0162 | 20 |
| 12 | 0.029 | 0.011 | 0.25 | 0.011 | 0.012 | 0.054 | 0.0159 | 36 |
| 13 | 0.030 | 0.009 | 0.24 | 0.013 | 0.014 | 0.064 | 0.0141 | 14 |
| 14 | 0.031 | 0.008 | 0.21 | 0.010 | 0.010 | 0.050 | 0.0135 | 27 |
| 15 | 0.022 | 0.010 | 0.30 | 0.012 | 0.011 | 0.042 | 0.0155 | 43 |
| 16 | 0.026 | 0.012 | 0.28 | 0.008 | 0.012 | 0.040 | 0.0152 | 26 |
| 17 | 0.033 | 0.011 | 0.25 | 0.010 | 0.009 | 0.034 | 0.0143 | 39 |
| 18 | 0.037 | 0.010 | 0.31 | 0.011 | 0.010 | 0.032 | 0.0148 | 3 |
| 19 | 0.034 | 0.013 | 0.24 | 0.009 | 0.013 | 0.041 | 0.0151 | 112 |

| | | | | | | | | |
|---|---|---|---|---|---|---|---|---|
| *Due to occurrence of slab crack in steel sheet No. 10 in continuous casting, operations thereafter were not performed. | | | | | | | | |

**Table 2**

| No. | Hot rolling coiling temperature (°C) | Continuous annealing soaking temperature (°C) | Continuous annealing soaking period (second) | Second cold rolling reduction ratio (%) |
|---|---|---|---|---|
| 1 | 582 | 668 | 21 | 11.5 |
| 2 | 589 | 685 | 21 | 9.8 |
| 3 | 575 | 698 | 10 | 8.3 |
| 4 | 598 | 621 | 23 | 10.6 |
| 5 | 552 | 605 | 49 | 14.9 |
| 6 | 563 | 654 | 22 | 12.7 |
| 7 | 584 | 620 | 23 | 13.1 |
| 8 | 571 | 683 | 21 | 11.1 |
| 9 | 591 | 667 | 21 | 10.9 |
| 10 | - | - | - | - |
| 11 | 604 | 644 | 22 | 9.2 |
| 12 | 585 | 598 | 24 | 12.2 |
| 13 | 587 | 703 | 15 | 14.0 |
| 14 | 592 | 683 | 9 | 12.5 |
| 15 | 566 | 672 | 52 | 10.3 |
| 16 | 570 | 658 | 22 | 7.8 |
| 17 | 581 | 631 | 23 | 15.5 |
| 18 | 590 | 689 | 21 | 13.3 |
| 19 | 588 | 690 | 21 | 10.1 |

| | | | | |
|---|---|---|---|---|
| *Due to occurrence of slab crack in steel sheet No. 10 in continuous casting, operations thereafter were not performed. | | | | |

The resin coated steel sheet obtained as described above was subjected to tensile testing. The tensile testing conforms to Metallic materials-Tensile testing defined in the document "JIS Z 2241", and strength of tension (tensile strength) was measured using a test piece for tensile testing having a size of JIS5. Moreover, the obtained resin coated steel sheet was subjected to Erichsen test. The Erichsen test conforms to Method of Erichsen cupping test defined in the document "JIS Z 2247", and an Erichsen value (a bulging height at which a penetration crack occurred) was measured using a test piece of 90 mm × 90 mm. Furthermore, a rivet for attaching an EOE tab was formed using the obtained resin coated steel sheet, and the rivet formability was evaluated. The rivet formation was performed by three phases of press working, and processing for reducing a diameter was performed after bulging to form a spherical-head-formed rivet having a diameter of 4.0 mm and a height of 2.5 mm. Occurrence of a crack in a rivet portion was evaluated as "C", occurrence of necking in a thickness direction, which is a previous stage leading to a crack, was evaluated as "B", and no occurrence of a crack or necking in a thickness direction was evaluated as "A". The obtained results are listed in Table 3.

**Table 3**

| No. | Tensile strength (MPa) | Erichsen value (mm) | Rivet formability | |
|---|---|---|---|---|
| 1 | 552 | 6.9 | A | Inventive Example |
| 2 | 535 | 7.4 | A | Inventive Example |
| 3 | 523 | 7.6 | A | Inventive Example |
| 4 | 539 | 7.0 | A | Inventive Example |
| 5 | 591 | 5.2 | A | Inventive Example |
| 6 | 557 | 6.5 | A | Inventive Example |
| 7 | 516 | 6.2 | A | Comparative Example |
| 8 | 592 | 4.8 | C | Comparative Example |
| 9 | 517 | 7.3 | A | Comparative Example |
| 10 | - | - | - | Comparative Example |
| 11 | 532 | 4.2 | C | Comparative Example |
| 12 | 595 | 4.8 | C | Comparative Example |
| 13 | 512 | 6.1 | A | Comparative Example |
| 14 | 603 | 4.9 | C | Comparative Example |
| 15 | 515 | 7.2 | A | Comparative Example |
| 16 | 517 | 7.9 | A | Comparative Example |
| 17 | 599 | 4.9 | C | Comparative Example |
| 18 | 564 | 6.0 | B | Comparative Example |
| 19 | 538 | 7.3 | B | Comparative Example |

| | | | | |
|---|---|---|---|---|
| *Due to occurrence of slab crack in steel sheet No. 10 in continuous casting, operations thereafter were not performed. | | | | |

As listed in Table 3, the steel sheets of Inventive Examples No. 1 to No. 6 are excellent in strength, and achieve tensile strength of not lower than 520 MPa that is required as an ultrathin steel sheet for cans. Moreover, they are also excellent in formability, and have an Erichsen value of not less than 5.0 mm that is required in EOE processing. Furthermore, even if the rivet formation is performed, no crack or necking in a thickness direction occurs. By contrast, each of the steel sheets of Comparative Examples No. 7 and No. 9 has such small C and N content that they are lacking in tensile strength. The steel sheet of Comparative Example No. 8 has such large C content that the formability is deteriorated by second cold rolling, resulting in the lack in Erichsen value and thus causing a crack in rivet formation.

The steel sheet of Comparative Example No. 10 has such large N content that a slab crack has occurred in continuous casting. Regarding the steel sheet of Comparative Example No. 11, the local elongation deteriorates because the coiling temperature after hot rolling is too high, resulting in the lack in Erichsen value and thus causing a crack in rivet formation. Regarding the steel sheet of Comparative Example No. 12, recrystallization is insufficient because the soaking temperature in continuous annealing is too low, resulting in the lack in Erichsen value and thus causing a crack in rivet formation. Regarding the steel sheet of Comparative Example No. 13, grain growth is excessive because the soaking temperature in continuous annealing is too high, resulting in the lack in tensile strength. Regarding the steel sheet of Comparative Example No. 14, recrystallization is insufficient because the soaking period in continuous annealing is too short, resulting in the lack in Erichsen value and thus causing a crack in rivet formation.

Regarding the steel sheet of Comparative Example No. 15, grain growth is excessive because the soaking period in continuous annealing is too long, resulting in the lack in tensile strength. The steel sheet of Comparative Example No. 16 is lacking in tensile strength because the second cold rolling reduction ratio is too small. Regarding the steel sheet of Comparative Example No. 17, work hardening becomes excessive because the second cold rolling reduction ratio is too high, resulting in the lack in Erichsen value and thus causing a crack in rivet formation. Regarding the steel sheet of No. 18 that is a Comparative Example, the thickness of the resin film coating the surface of the steel sheet is too thin, and thus the effects thereof are not sufficiently exerted in rivet formation, causing a necking in a thickness direction before leading to a crack. Regarding the steel sheet of No. 19 that is a Comparative Example, the thickness of the resin film coating the surface of the steel sheet is too thick, and thus the deformation amount of the steel sheet is increased in rivet formation, causing a necking in a thickness direction before leading to a crack.

Based on the above, it was confirmed that according to the steel sheets of the inventive examples, it is possible to obtain a high strength and high formability steel sheet for easy open ends of cans having tensile strength of not lower than 520 MPa and an Erichsen value of not less than 5.0 mm.

The embodiments to which the present invention made by the inventors are applied have been described. However, the present invention is not limited by the description that forms a part of the disclosure of the present invention in the embodiments. That is, other embodiments, examples, and operation technologies that are made based on the present embodiments by a person skilled in the art, etc. are all included in the scope of the present invention as long as these are within the scope of the appended claims.

### Industrial Applicability

According to the present invention, it is possible to provide a high strength and high formability steel sheet for easy open ends of cans having tensile strength of not lower than 520 MPa and an Erichsen value of not less than 5.0 mm.

## Claims

1. A high strength and high formability steel sheet for easy open ends of cans having a tensile strength in a rolling direction of not less than 520 MPa, and an Erichsen value of not less than 5.0 mm, which is obtainable by:
forming a slab by continuously casting a steel including, in mass%:
greater than 0.020% and less than 0.040% of C;
not less than 0.003% and not greater than 0.100% of Si;
not less than 0.10% and not greater than 0.60% of Mn;
not less than 0.001% and not greater than 0.100% of P;
not less than 0.001% and not greater than 0.020% of S;
not less than 0.005% and not greater than 0.100% of Al;
greater than 0.0130% and not greater than 0.0170% of N; and
a remainder being Fe and inevitable impurities;
performing hot rolling at a slab reheating temperature of not lower than 1150°C;
coiling at a temperature of not higher than 600°C;
thereafter performing first cold rolling;
thereafter performing continuous annealing at a soaking temperature of 600 to 700°C for a soaking period of 10 to 50 seconds; and
thereafter performing second cold rolling at a reduction ratio of 8.0 to 15.0%,
the high strength and high formability steel sheet being **characterized by** comprising a resin film layer with a thickness of 5 to 100 µm at least on a side to be an inner surface of a can.

2. A method of manufacturing a high strength and high formability steel sheet for easy open ends of cans, the method comprising:
forming a slab by continuously casting a steel including, in mass%:
greater than 0.020% and less than 0.040% of C;
not less than 0.003% and not greater than 0.100% of Si;
not less than 0.10% and not greater than 0.60% of Mn;
not less than 0.001% and not greater than 0.100% of P;
not less than 0.001% and not greater than 0.020% of S;
not less than 0.005% and not greater than 0.100% of Al;
greater than 0.0130% and not greater than 0.0170% of N; and
a remainder being Fe and inevitable impurities;
performing hot rolling at a slab reheating temperature of not lower than 1150°C;
coiling at a temperature of not higher than 600°C;
thereafter performing first cold rolling;
thereafter performing continuous annealing at a soaking temperature of 600 to 700°C for a soaking period of 10 to 50 seconds;
thereafter performing second cold rolling at a reduction ratio of 8.0 to 15.0%;
attaching a resin film with a thickness of 5 to 100 µm at least on a side to be an inner surface of a can after forming a surface treatment film by an electrolytic process; and
manufacturing a steel sheet having a tensile strength in a rolling direction of not less than 520 MPa and an Erichsen value of not less than 5.0 mm.

## Patentansprüche

1. Hochfestes und hochverformbares Stahlblech für Aufreißdeckel von Dosen mit einer Zugfestigkeit in Walzrichtung von nicht weniger als 520 MPa und einem Erichsen-Wert von nicht weniger als 5,0 mm, das erhältlich ist durch:
Formen einer Bramme durch kontinuierliches Gießen eines Stahls, in Massen-% enthaltend:
mehr als 0,020% und weniger als 0,040% C;
nicht weniger als 0,003% und nicht mehr als 0,100% Si;
nicht weniger als 0,10% und nicht mehr als 0,60% Mn;
nicht weniger als 0,001% und nicht mehr als 0,100% P;
nicht weniger als 0,001% und nicht mehr als 0,020% S;
nicht weniger als 0,005% und nicht mehr als 0,100% Al;
mehr als 0,0130% und nicht mehr als 0,0170% N; und
einen Rest aus Fe und unvermeidbaren Verunreinigungen;
Durchführen von Warmwalzen bei einer Nacherwärmungstemperatur der Bramme von nicht niedriger als 1150°C;
Aufrollen bei einer Temperatur von nicht höher als 600°C;
anschließendes Durchführen eines ersten Kaltwalzens;
anschließendes Durchführen von kontinuierlichem Glühen bei einer Haltetemperatur von 600 bis 700°C für eine Haltedauer von 10 bis 50 Sekunden; und
anschließendes Durchführen eines zweiten Kaltwalzens bei einem Reduktionsverhältnis von 8,0 bis 15,0%,
wobei das hochfeste und hochverformbare Stahlblech dadurch charakterisiert ist, dass es eine Harzfolienschicht mit einer Dicke von 5 bis 100 µm mindestens auf einer Seite, die eine innere Oberfläche einer Dose darstellt, umfasst.

2. Verfahren zur Herstellung eines hochfesten und hochverformbaren Stahlblechs für Aufreißdeckel von Dosen, das Verfahren umfassend:
Formen einer Bramme durch kontinuierliches Gießen eines Stahls, in Massen-% enthaltend:
mehr als 0,020% und weniger als 0,040% C;
nicht weniger als 0,003% und nicht mehr als 0,100% Si;
nicht weniger als 0,10% und nicht mehr als 0,60% Mn;
nicht weniger als 0,001% und nicht mehr als 0,100% P;
nicht weniger als 0,001% und nicht mehr als 0,020% S;
nicht weniger als 0,005% und nicht mehr als 0,100% Al;
mehr als 0,0130% und nicht mehr als 0,0170% N; und
einen Rest aus Fe und unvermeidbaren Verunreinigungen;
Durchführen von Warmwalzen bei einer Nacherwärmungstemperatur der Bramme von nicht niedriger als 1150°C;
Aufrollen bei einer Temperatur von nicht höher als 600°C;
anschließendes Durchführen eines ersten Kaltwalzens;
anschließendes Durchführen von kontinuierlichem Glühen bei einer Haltetemperatur von 600 bis 700°C für eine Haltedauer von 10 bis 50 Sekunden;
anschließendes Durchführen eines zweiten Kaltwalzens bei einem Reduktionsverhältnis von 8,0 bis 15,0%;
Anbringen einer Harzfolie mit einer Dicke von 5 bis 100 µm mindestens auf einer Seite, die nach dem Bilden einer Oberflächenbehandlungsfolie mittels eines elektrolytischen Prozesses eine innere Oberfläche einer Dose darstellt; und
Herstellen eines Stahlblechs mit einer Zugfestigkeit in Walzrichtung von nicht weniger als 520 MPa und einem Erichsen-Wert von nicht weniger als 5,0 mm.

## Revendications

1. Tôle d'acier facilement façonnable et de résistance élevée pour ouvrir facilement les extrémités de boîtes ayant une résistance à la traction dans une direction de laminage de pas moins de 520 MPa, et une valeur d'Erichsen de pas moins de 5,0 mm, qui peut être obtenue par :
la formation d'une brame par la coulée continue d'un acier incluant, en % en masse :
plus de 0,020 % et moins de 0,040 % de C ;
pas moins de 0,003 % et pas plus de 0,100 % de Si ;
pas moins de 0,10 % et pas plus de 0,60 % de Mn ;
pas moins de 0,001 % et pas plus de 0,100 % de P ;
pas moins de 0,001 % et pas plus de 0,020 % de S ;
pas moins de 0,005 % et pas plus de 0,100 % d'Al ;
plus de 0,0130 % et pas plus de 0,0170 % de N ; et
le reste étant Fe et des impuretés inévitables ;
la mise en oeuvre d'un laminage à chaud à une température de réchauffage de brame de pas moins de 1150 °C ;
un enroulement à une température de pas plus de 600 °C ;
ensuite la mise en oeuvre d'un premier laminage à froid ;
ensuite la mise en oeuvre d'un recuit continu à une température de trempe de 600 à 700 °C pendant une période de trempe de 10 à 50 secondes ; et
ensuite la mise en oeuvre d'un second laminage à froid à un rapport de réduction de 8,0 à 15,0 %,
la tôle d'acier facilement façonnable et de résistance élevée étant **caractérisée en ce qu'**elle comprend une couche de film de résine ayant une épaisseur de 5 à 100 µm au moins sur une face pour être une surface interne d'une boîte.

2. Procédé de fabrication d'une tôle d'acier facilement façonnable et de résistance élevée pour ouvrir facilement les extrémités de boîtes, le procédé comprenant :
la formation d'une brame par la coulée continue d'un acier incluant, en % en masse :
plus de 0,020 % et moins de 0,040 % de C ;
pas moins de 0,003 % et pas plus de 0,100 % de Si ;
pas moins de 0,10 % et pas plus de 0,60 % de Mn ;
pas moins de 0,001 % et pas plus de 0,100 % de P ;
pas moins de 0,001 % et pas plus de 0,020 % de S ;
pas moins de 0,005 % et pas plus de 0,100 % d'Al ;
plus de 0,0130 % et pas plus de 0,0170 % de N ; et
le reste étant Fe et des impuretés inévitables ;
la mise en oeuvre d'un laminage à chaud à une température de réchauffage de brame de pas moins de 1150 °C ;
un enroulement à une température de pas plus de 600 °C ;
ensuite la mise en oeuvre d'un premier laminage à froid ;
ensuite la mise en oeuvre d'un recuit continu à une température de trempe de 600 à 700 °C pendant une période de trempe de 10 à 50 secondes ;
ensuite la mise en oeuvre d'un second laminage à froid à un rapport de réduction de 8,0 à 15,0 % ;
la fixation d'un film de résine ayant une épaisseur de 5 à 100 µm au moins sur une face pour être une surface interne d'une boîte après la formation d'un film de traitement de surface par un procédé électrolytique ; et
la fabrication d'une tôle d'acier ayant une résistance à la traction dans une direction de laminage de pas moins de 520 MPa et une valeur d'Erichsen de pas moins de 5,0 mm.
